# EUROPEAN PATENT SPECIFICATION

(11) **EP 2 129 812 B1**
(45) Date of publication and mention of the grant of the patent: **17.04.2013**
(21) Application number: 08717723.4
(22) Date of filing: 13.03.2008
(51) Int. Cl.: C23C 28/02, F01D 5/28, F04D 29/02, F01D 25/00, C23C 4/06, C23C 4/12, C23C 26/02, C23F 13/02

(54) **TURBOMACHINE BLADE WITH EROSION AND CORROSION PROTECTIVE COATING AND METHOD OF MANUFACTURING THE SAME**
TURBOMASCHINENSCHAUFEL MIT EROSIONS- UND KORROSIONSSCHUTZBESCHICHTUNG UND HERSTELLUNGSVERFAHREN DAFÜR
PALE DE TURBOMACHINE AVEC REVÊTEMENT DE PROTECTION CONTRE L'ÉROSION ET LA CORROSION, ET PROCÉDÉ DE FABRICATION DE CETTE DERNIÈRE

(30) Priority: 27.03.2007 DE 102007015310; 20.06.2007 US 765599
(43) Date of publication of application: 09.12.2009
(73) Proprietor: Alstom Technology Ltd, 5400 Baden (CH)
(72) Inventor: BARRIL, Marie-Gilles, CH-5413 Birmenstorf (CH); GRASSO, Piero-Daniele, CH-8165 Oberweningen (CH); STANKOWSKI, Alexander, CH-5301Siggenthal-Station (CH)
(86) International application number: PCT/EP2008/052979
(87) International publication number: WO 2008/116757

(56) References cited:
- EP-A- 1 666 633
- EP-A- 1 700 929
- EP-A- 1 826 363
- WO-A1-2006/094935
- CA-C- 2 039 944
- GB-A- 2 241 961
- US-A- 4 125 646
- US-A- 4 537 632
- US-A- 5 279 649
- US-A- 5 747 163
- US-A1- 2002 197 152
- US-A1- 2006 018 760
- US-A1- 2007 017 958

## Description

### FIELD OF THE INVENTION

The present invention relates to a turbomachine blade, in particular to a compressor blade for use in a gas turbine engine. The present invention also relates to a method of manufacturing a turbomachine blade, the method comprising the step of depositing a corrosion and erosion protective coating on the turbomachine blade body.

### BACKGROUND OF THE INVENTION

It is known from the state of the art that turbomachine blades, in particular compressor blades, which are made of metallic material such as stainless steel, are susceptible to corrosion, in particular pitting corrosion.

Pitting corrosion is a form of localized corrosion that leads to the creation of small holes in the metallic material based on galvanic corrosion. As is known, pitting corrosion can be initiated by small surface defects such as scratches, holes or local changes of the composition of the material and it may be aggravated by salt deposits and humidity during operation or stand still of the turbine engine.

Due to water droplets and particulate matter impacting on the leading edge area of compressor blades in a gas turbine pitting corrosion is a frequently occuring degradation mechanism for compressor blading.

Moreover, pitting corrosion is extremely insidious as it causes only little loss of material with small effects on the metal surface. However, it causes serious damages in the deep structure of the metal. When corrosion pits reach a certain depth, particularly in the leading edge area of the blade, they can lead to the formation of cracks, which may finally result in blade failure due to high cyclic fatigue (HCF).

In order to avoid pitting corrosion, it is known to deposit corrosion protective layers on the blade body material. In recent years, sacrificial slurry coatings have become rather popular for use as corrosion protective layers, in particular for use in the front stages in compressor blading. These coatings are sacrificial because they are attacked instead of the blading material. However, it has become apparent that even sacrificial slurry coatings are prone to degradation in highly erosive conditions as they typically can be found at the leading edges of compressor blades due to water droplets and particles that hit the blades very hard. Because of local loss of the coating's erosion resistant property, corrosion of the leading edge area may occur.

### SUMMARY OF THE INVENTION

In light of the above, it is an object of the invention to provide a turbomachine blade that has an improved corrosion and erosion protective coating to enable a longer working life of the blade. It is another object of the invention to provide a method of manufacturing such a turbomachine blade.

The afore-mentioned objects are achieved by a method of manufacturing a turbomachine blade according to claim 1

According to one aspect of the invention a turbomachine blade, which may be a compressor blade, comprises a blade body and a corrosion and erosion protective multilayered coating bonded to the blade body. The multilayered coating comprises an erosion resistant first layer and a sacrificial second layer with the latter one being provided in overlying relationship to the first one.

Preferably, the erosion resistant first layer is selected so as to provide erosion resistance against water droplets or particles impacting on it. In case the blade body is made of stainless steel, the first layer may be selected so as to provide stainless steel corrosion resistance as well.

According to a further aspect of the invention, the erosion resistant first layer is deposited so that it covers at least an corrosion (and erosion) critical area of the blade body such as a leading edge area of the blade. However, it may be preferred that the first layer exclusively covers the erosion critical area of the blade body and does not cover any area of the blade body not belonging to the erosion critical area.

Depending on the severity of the erosion attack, the first layer preferably covers an area of up to 30% of the chord length starting from the leading edge towards the suction and pressure sides of the blade that is to say towards the trailing edge of the blade. The first layer may cover an area of from 5 to 30% of the chord length starting from the leading edge towards the trailing edge. But it may also cover an area of up to 60% or more of the chord length starting from the leading edge towards the trailing edge in case of a stronger impact of particulate matter and water droplets.

The sacrificial second layer is deposited so that it covers the first layer at least totally. However, it may be preferred that the sacrificial second layer covers the blade body totally.

In the turbomachine blade of the present invention, it may be preferred that the first layer is sandwiched between the blade body and the second layer. Accordingly, the first layer is arranged so as to be an intermediate layer between the blade body and the second layer in an adjacent relationship relative to the blade body and the second layer.

In the present invention, the first layer may have a layer thickness in the range of from 50 to 100 micrometer (µm) while the second layer may have a layer thickness in the range of from 50 to 100 micrometer (µm) resulting in a total protective coating thickness in the range of from 100 to 200 micrometer (µm) with a maximum total thickness of 200 micrometer (µm).

The first layer is selected so as to be a braze tape or a foil containing a matrix of braze alloy with an erosion resistant filler material essentially consisting of abrasive particles. The braze alloy may be a Silver (Ag)-based alloy or an Aluminum (Al)-based alloy or any other suitable alloy. The erosion resistant filler may be selected so as to consist of one or more filler materials selected from the group consisting of Al₂O₃, WC, CrC or any other suitable erosion resistant material. The filler content may range from 60 to 90 Vol.% of the first layer and sizes of the filler particles may range from 10 to 30 micrometer (µm).

In the present invention, a roughness of the first layer is made to be smaller than 2.3 micrometer (µm) depending on the first layer deposition technique.

The first layer material is deposited using the tape/foil brazing technique.

In the present invention, the second layer is a sacrificial slurry coating. The sacrificial slurry coating for consists of a closely packed aluminum-filled chromate/phophate basecoat that is sealed with a chemically inert chromate/phosphate topcoat on top of the basecoat. Preferably, a roughness of the sacrificial slurry coating is made to be smaller than 1.6 micrometer (µm) depending on the first layer deposition technique.

According to a further aspect of the invention, a method of manufacturing above-described turbomachine blade comprises the steps of:
- providing the blade body, followed by
- a two-step process of depositing the corrosion and erosion protective coating on the blade body, namely
- a first deposition step of depositing an erosion and corrosion resistant first layer in order to cover at least the corrosion critical area, in particular the leading edge area of the blade body, and a subsequent
- second deposition step of depositing a sacrificial second layer over the first layer in order to cover at least the first layer and preferably the whole blade body.

Deposition of the second layer may be effected using one or more standard spraying techniques. The first layer is deposited on the base material by tape/foil brazing technique.

In a turbomachine blade having a blade body made of stainless steel, the first layer material is deposited using tape/foil brazing technique. Upon doing so, brazing temperatures used may not exceed a tempering temperature of the stainless steel blade body material.

The above and still further objects, features and advantages of the present invention will become apparent upon consideration of the following detailed description of an embodiment thereof.

### BRIEF DESCRIPTION OF THE DRAWINGS

- FIG. 1: schematically depicts a transversal sectional view of an embodiment of a compressor blade provided with a corrosion protective coating according to the present invention;
- FIG. 2: schematically depicts a method of manufacturing the compressor blade shown in FIG. 1.

### DETAILED DESCRIPTION OF AN EMBODIMENT

An embodiment of the present invention will be described in detail below with reference to the accompanying drawings.

Reference is now made to FIG. 1 that shows a transversal sectional view of an embodiment of a compressor blade for a gas turbine which is provided with a corrosion protective coating according to the present invention.

A compressor blade 1 comprises a blade body (substrate) 2 that for instance is made of stainless steel. Due to its typical body shape, the blade body has a major bulged pressure side 7 (in FIG. 1 upper side) and a minor bulged suction side 6 (in FIG. 1 lower side) both of which are formed to converge in a dull leading edge 8 and an acute trailing edge 9 of the blade body 2. The outer surface 10 of the blade body 2 is covered with a corrosion and erosion protective bilayer coating 11 that is bonded thereto.

The bilayer coating 11 comprises a lower erosion resistant first layer 3 that is provided on the surface of blade body 2 and arranged in a leading edge area 5 surrounding the leading edge 8 on both the suction side 6 and the pressure side 7 of the blade body 2. The first layer 3 covers a covering area of up to 60% of the airfoil chord length starting from the leading edge 8 towards the trailing edge 9 of the blade body 2. In FIG. 1, the airfoil chord length can be identified by the outer surface 10 of the blade body 2.

The erosion resistant first layer 3 material is selected so as to provide erosion resistance against water droplets or particles impacting on the leading edge 8 area 5.

To this end the first layer 3 is a braze tape or foil containing a matrix of braze alloy, such as a Silver (Ag)-based alloy or an Aluminium (Al)-based alloy, and an erosion resistant filler material, such as Al₂O₃, WC and CrC. The filler content ranges from 60 to 90 Vol.-% of the first layer 3 and sizes of the filler particles preferably range from 10 to 30 micrometers (µm). The layer thickness of the first layer 3 preferably ranges from 50 to 100 µm.

The bilayer coating 11 further comprises an upper sacrificial second layer 4 that covers (is deposited on) the first layer 3 and the remaining non-covered parts of the blade body 2 surface 10. The first layer 3 is sandwiched between the blade body 2 and the second layer 4. The second layer 4 is a sacrificial slurry coating that consists of a closely packed aluminum-filled chromate/phosphate basecoat that is sealed with a chemically inert chromate/phosphate topcoat on top of the basecoat (both basecoat and topcoat are not further detailed in FIG. 1). The second layer 4 has a layer thickness ranging from 50 to 100 µm resulting in a total bilayer coating 11 thickness ranging from 100 to 200 µm.

Reference is now made to FIG. 2 that schematically depicts a method of manufacturing the compressor blade 1 shown in FIG. 1, the method comprising two deposition steps for depositing the corrosion protective bilayer coating 11.

After a non-covered blade body 2 has been provided (step I), the erosion resistant first layer 3 is deposited on the surface (outer skin) 10 of the blade body 2 in the leading edge 8 area 5 (step II). In a further step, starting from a partly covered blade body 2 (step II), the sacrificial slurry second layer 4 is deposited on both the first layer 3 and the remaining non-covered portions of the blade body 2 surface 10 to thereby coat the whole blade body 2 (step III).

To deposit the first layer 3 on the base material tape/foil brazing technique is used. Deposition of the second layer may be effected using one or more standard spraying techniques.

The deposition techniques may be selected so as to achieve a roughness of both the erosion resistant first layer 3 and sacrificial slurry second layer 4 of less than 2.3 µm.

As can be seen from the above, by bonding a corrosion protective bilayer coating 11 on the outer surface 10 of the blade body 2 the working life of the blade 1 can be increased significantly because of the provision of an increased local erosion and corrosion protection and the risk of premature failure due to pitting corrosion attack is reduced. The bilayer coating and the process for coating can be realized with low costs. By restricting the erosion resistant first layer 3 to the leading edge area 5 of the blade body 2 that is particularly endangered by early erosion, manufacturing costs and time can be reduced additionally.

Compressor blades with a bilayer structure of the present invention are reconditionable.

### Reference list

- 1: Turbomachine blade
- 2: Blade body
- 3: Erosion and corrosion resistant first layer
- 4: Sacrificial second layer
- 5: Leading edge area
- 6: Suction side
- 7: Pressure side
- 8: Leading edge
- 9: Trailing edge
- 10: Blade body surface
- 11: Corrosion protective bilayer coating

## Claims

1. A method of manufacturing a turbomachine blade comprising the steps of:
- providing a blade body (2);
- using a brazing technique to deposit an erosion and corrosion resistant first layer (3) on the blade body (2) so as to cover at least a corrosion critical area (5), in particular a leading edge area, of the blade body (2),
- wherein the brazing technique uses a braze tape or foil containing a matrix of braze alloy with an erosion resistant filler consisting of abrasive particles
- followed by
- depositing a sacrificial second layer (4) over the first layer so as to cover at least the first layer (3) wherein said second layer (4) is a sacrificial slurry coating that consists of a closely packed aluminum-filled chromate/phosphate basecoat that is sealed with a chemically inert chromate/phosphate topcoat.

## Patentansprüche

1. Verfahren zum Herstellen einer Turbomaschinenschaufel, das die folgenden Schritte umfasst:
- Bereitstellen eines Schaufelkörpers (2);
- Verwenden einer Hartlöttechnik zum Abscheiden einer erosions- und korrosionsbeständigen ersten Schicht (3) auf dem Schaufelkörper (2), um mindestens einen korrosionskritischen Bereich (5), insbesondere einen Vorderkantenbereich, des Schaufelkörpers (2) zu bedecken,
- wobei die Hartlöttechnik ein Hartlötband oder eine Hartlötfolie verwendet, das oder die eine Matrix aus Hartlötlegierung mit einem erosionsbeständigen Füllmittel enthält, das aus Schleifpartikeln besteht,
- gefolgt von
- Abscheiden einer zweiten Opferschicht (4) über der ersten Schicht, um mindestens die erste Schicht (3) zu bedecken, wobei die zweite Schicht (4) eine Opferaufschlämmungsbeschichtung ist, die aus einer dicht gepackten aluminiumgefüllten Chromat-/Phosphat-Grundschicht besteht, die mit einer chemisch inerten Chromat-/Phosphat-Deckschicht versiegelt ist.

## Revendications

1. Procédé de fabrication d'une aube de turbomachine, le procédé comportant les étapes qui consistent à :
prévoir un corps d'aube (2),
utiliser une technique de brasage pour déposer sur le corps d'aube (2) une première couche (3) qui résiste à l'érosion et à la corrosion en recouvrant au moins une zone (5) critique vis-à-vis de la corrosion et en particulier une zone de bord d'attaque du corps d'aube (2),
la technique de brasage utilisant un ruban ou une feuille de brasure contenant une matrice d'alliage de brasure dotée d'une charge constituée de particules abrasives résistant à l'érosion,
avec ensuite
le dépôt d'une deuxième couche sacrifiée (4) sur la première couche de manière à couvrir au moins la première couche (3), ladite deuxième couche (4) étant un revêtement sacrifié de suspension constitué d'un revêtement compact de base au chromate/phosphate chargé en aluminium, fermé hermétiquement par un revêtement supérieur chimiquement inerte au chromate/phosphate.
